

## UNITED STATES PATENT OFFICE

2,233,683

## LUBRICANT

William Alvah Smith, Hamburg, N. Y.

No Drawing. Application August 9, 1935.  
Serial No. 35,516

20 Claims. (Cl. 252—54)

This invention relates to lubricants, and has for an object to obtain a lubricant having uniform lubricating characteristics such as high load carrying capacity, and shock resistance, and low power consumption characteristics.

Another object of the invention is to provide an improved method of preparing lubricants, with which uniformity in the product and the most desirable characteristics may be consistently obtained.

This application is a continuation-in-part of and relates to an improvement upon the inventions disclosed in my prior copending applications Ser. No. 643,897 filed November 22, 1932, and Ser. 15 No. 15,635 filed April 10, 1935. In those prior applications I have disclosed a lubricant which possesses high load carrying capacity and shock resistance, and low power consumption characteristics. This lubricant comprises essentially 20 a mineral lubricating oil compounded with a minor proportion of halogenated hydrocarbons, which may be aliphatic, aromatic, or alicyclic, and a minor proportion of saponifiable, oxygen containing organic compounds. In quantity production I found, however, that different batches 25 of my lubricant, of apparently identical composition, differed in lubricating characteristics.

I have discovered that uniformity, as well as enhanced results can be obtained by heating to 30 high temperatures (for example, 200° C.) preferably with agitation, for a short but sufficient period of time, such as fifteen minutes, either the components of the improved lubricant, separately or in groups and mixing preferably while hot or 35 above room temperatures, or the compounded lubricant mixture. For example, an S. A. E. #90 gear lubricant containing 8% of chlorinated naphthalene (carrying about 63% chlorine), 2% of oxidized petroleum acids, and 1/4% of alpha monochlornaphthalene apparently will go together completely at 110° C. but the mixture at a load of 200 pounds gage on a Floyd lubricant tester sometime shows scratching of the test pieces. When heated to 200° C. for fifteen 40 minutes, with stirring, the same lubricant carries 200 pounds for five minutes, which may be followed by 325 pounds for five minutes, without scratching of the test pieces. The load may then be increased to 600 pounds, whereupon the test 45 piece will begin to extrude, the bearing surfaces being afterward found to be perfectly burnished and free from scratches. Furthermore, these results can be duplicated repeatedly.

Certain chlorinated organic compounds (for example aliphatics, alicyclics, etc.) will not with-

stand these high temperatures without decomposition, and lubricant plants are not ordinarily equipped for developing such high temperatures. After experimentation, therefore, I have found that equal results may be obtained at lower temperatures, for example 100° C., by prolonging the heating time for the lubricant, and its components. In one case, heating sixteen hours at 110° C. gave satisfactory results. In other cases still lower temperatures are desirable and practicable. 5 At these relatively low temperatures, a vacuum should preferably be used. For example, approximately twenty-nine inches of vacuum applied at approximately 80° C. for a sufficient time will develop the desired characteristics. 10

In all of the above examples, the end result is the same—to develop uniform and high qualities, and I have found that the use of heat under properly controlled conditions develops these desired characteristics. Whether the result secured 15 by this heat treatment is because of the elimination of traces of moisture or some other deleterious constituent, either by volatilization or precipitation, or by the production of a physical coordination or chemical union between the components of 20 the lubricant, or a combination of these factors, I am unable at this time to state definitely, but the resultant lubricants have maximum pressure 25 and minimum friction characteristics for the particular combinations used, with little or no change 30 in viscosity.

The heat treatment with agitation appears to homogenize the mixture. The degree of heat selected for any particular compound is preferably one which is below the temperature at which the 35 ingredients or agents or any of them become unstable. Since the duration of the heating may vary to some extent, depending upon the temperatures used, I prefer to continue the heating in each case until samples of the homogenized and 40 treated mixture taken at successive intervals during the heating or homogenizing operation, when tested on a lubricant tester, show that the mixture has developed the desired and uniform lubricating characteristics, as determined by reference to a standard specification. When the 45 components are heated separately the heating is continued until samples taken at intervals and homogenized with the other components give similar test indications when the homogenized 50 test blends are tested.

While I prefer to mix all the ingredients and homogenize the mixture with heat until the mixture possesses the desired and uniform lubricating characteristics as above explained, I have found 55

that beneficial effects may be obtained by separately heat treating the oil and added agents or ingredients, and then mixing the oil with the agent or agents while hot. The mixture may then be further homogenized, with beneficial results, by reheating until the desired characteristics are obtained.

While the reason for this improvement, as explained above, is not definitely known, I believe that the improvement may be due to the elimination of moisture from the oil and the ingredients, the theory being that any moisture present in the mixture may form films which separate the material into globules which hinder chemical union or cooperation of the components or that do not coalesce as readily as if the film were not present, producing a result comparable with a suspension or emulsion which is liable to break down and allow the ingredients to separate.

While the free moisture can be eliminated in any suitable manner, such as by subjecting the materials to well known chemical moisture removing agents, I have found that the heat treatment is the simplest and most satisfactory method of accomplishing the purpose, because the solutions are formed most readily under the action of heat, and the homogenizing or chemical union of the mixture proceeds more rapidly and satisfactorily while the mixture is heated. Therefore, I simplify the procedure by utilizing the heat and agitation, not only to remove the free moisture but also to accelerate the solution of the ingredients in the oil and homogenize and/or chemically unite the mixture. If the mixture is not heated in order to blend or homogenize the ingredients, or if the free moisture is not eliminated, the added ingredients or agents tend to separate out when the mixture is quiescent in some cases.

In my prior applications hereabove referred to, I have disclosed the mixing of a major proportion of a mineral lubricating oil with a minor proportion of a substantially neutral body of oil film strengthening, oil soluble hydrocarbon having a halogen, such as chlorine, in chemical combination therewith, such body being substantially non-volatile at ordinary temperatures, and a minor proportion of another body of friction reducing, oil soluble organic compound having oxygen in saponifiable chemical combination therewith. As an example of a neutral body of hydrocarbon I have mentioned chlorinated naphthalenes, chlorinated diphenyls, chlorinated naphthalenes and chlorinated paraffines to be particularly satisfactory.

Among the friction reducing compounds which may be employed are castor oil, oleic acid, stearic acid, lard oil and "Alox." The substances available under the name "Alox" are manufactured on a commercial scale and are available in the open market under the name "Alox." They are obtained by the controlled oxidation of paraffine hydrocarbons or acids and contain a variety of compounds which are believed to include lactones, internal anhydrides of hydroxylated compounds, ketones, ketone alcohols, fatty acids, aldehydes, and esters. Such substances are disclosed in U. S. Patents to Burwell No. 1,690,769 granted November 6, 1928, and No. 1,863,004 granted June 14, 1932. Reference to those patents may be had for further identification of materials known under the name "Alox."

While the best results are obtained by heating the mixture of the oil and the added agents,

I have found that beneficial effects can also be obtained by the heat treatment separately of the oil and the "Alox" or other friction reducing body, or of the chlorinated hydrocarbon, and then their mixture while hot, or, if desired, any two of them may be heated and then mixed while hot with the other agent or with the oil. I have also found that the heat treatment improves the solvent action of the oil for the friction reducing agent and the chlorinated product which may be added, and that this improvement persists after the oil has returned to ordinary temperatures.

I am aware that it is old in the art to heat chlorinated aliphatic hydrocarbons to a temperature of approximately 300° F. in order to remove hydrochloric acid which is unstable at that temperature, but to the best of my knowledge and belief no one heretofore has ever treated the oil and any or all of the ingredients either separately or together in the manner hereinabove disclosed in order to improve the lubricating characteristics of the mixture. It is noted, however, that according to this invention, there is no condensation product or Friedel-Kraft operation, because there is no production of free hydrochloric acid.

It will be understood that various changes in the steps, details and materials, which have been herein described by way of example, in order to explain the nature of the invention, may be made by those skilled in the art within the principle and scope of the invention, as expressed in the appended claims.

I claim as my invention:

1. In the manufacture of lubricants in which a halogenated hydrocarbon film-strength increasing agent and an oxygen bearing friction reducing agent, are added to increase the effectiveness of the lubricant, the method of insuring uniform and maximum effectiveness of the lubricant mixture which comprises heating the lubricant and at least one of the agents of the mixture under conditions of temperature and pressure and for a period of time which will eliminate any free moisture present in the lubricant and the agents that are heated, and homogenizing the mixture while hot.

2. In the manufacture of lubricants, in which a halogenated hydrocarbon film-strength increasing agent and an oxygen bearing friction reducing agent, are added to a lubricant in order to increase the effectiveness of the lubricant, the method of insuring uniform and maximum effectiveness of the lubricant mixture, which comprises removing free moisture from the lubricant and each of said added agents, and homogenizing the mixture while hot.

3. In the manufacture of lubricants, in which a halogenated hydrocarbon film-strength increasing agent and an oxygen bearing friction reducing agent, are added to a lubricant in order to increase the effectiveness of the lubricant, the method of insuring uniform and maximum effectiveness of the lubricant mixture, which comprises heating the lubricant and at least one of the agents of the mixture under conditions of temperature which will eliminate any free moisture present, and which temperature is below that at which the lubricant and any agent of the mixture become unstable, and homogenizing the mixture while hot.

4. In the manufacture of lubricants in which a halogenated hydrocarbon film-strength increasing agent and an oxygen bearing friction

- reducing agent, are added to increase the effectiveness of the lubricant, the method of insuring uniform and maximum effectiveness of the lubricant mixture which comprises heating the lubricant and at least one of the agents of the mixture after mixing of the same, under conditions of temperature and pressure and for a period of time which will eliminate any free moisture present in the lubricant and the agents 10 that are heated, and homogenizing the mixture while hot.
5. In the manufacture of lubricants, in which a halogenated hydrocarbon film-strength increasing agent and an oxygen bearing friction reducing agent are added to a lubricant in order to increase the effectiveness of the lubricant, the method of insuring uniform and maximum effectiveness of the lubricant mixture, which comprises mixing the lubricant with one of said 20 agents under anhydrous conditions, and homogenizing the mixture while hot until the agent is thoroughly blended throughout the lubricant and does not materially separate therefrom upon standing, and adding the other agent.
25. 6. In the manufacture of lubricants, in which a halogenated hydrocarbon film-strength increasing agent and an oxygen bearing friction reducing agent are added to a lubricant in order to increase the effectiveness of the lubricant, the method of insuring uniform and maximum effectiveness of the lubricant mixture, which comprises subjecting the lubricant and the added agents to heat under such pressure conditions and for such period of time as will eliminate 30 any free moisture present in the lubricant and the agents, but with the temperature below that at which the mixture and the components thereof become unstable, and homogenizing the mixture while hot.
40. 7. In the manufacture of lubricants to obtain a compound of high film strength and lower coefficient of friction over a significant range of working conditions than any one of its constituents or any two of its constituents combined, the method which comprises heating a major proportion of a lubricating oil, a minor proportion of a substantially neutral body of oil film strengthening, oil soluble hydrocarbon having halogen in chemical combination therewith, and 45 a minor proportion of another body of friction reducing oil soluble organic compound having oxygen in saponifiable chemical combination therewith, under conditions of temperature and pressure and for a period of time which would eliminate free moisture in any of the constituents, and homogenizing the mixture.
50. 8. In the manufacture of lubricants to obtain a compound of high film strength and lower coefficient of friction over a significant range of working conditions than any one of its constituents or any two of its constituents combined, the method which comprises heating together a major proportion of a mineral lubricating oil, a minor proportion of a friction reducing, oil 55 soluble organic compound having oxygen in saponifiable chemical combination therewith, and a minor proportion of another and substantially neutral body of oil film strengthening, oil soluble hydrocarbon having halogen in chemical combination therewith, until tests on a lubricant tester of samples thereof taken at successive intervals during the heating show maximum and substantially uniform film strength and minimum and uniform friction characteristics.
70. 9. In the manufacture of lubricants to obtain a compound of high film strength and lower coefficient of friction over a significant range of working conditions than any one of its constituents or any two of its constituents combined, the method which comprises heating a major proportion of a mineral lubricating oil, and a minor proportion of a friction reducing oil soluble organic compound having oxygen in saponifiable chemical combination therewith, and homogenizing the mixture with a halogenated hydrocarbon.
10. In the manufacture of lubricants to obtain a compound of high film strength and lower coefficient of friction over a significant range of working conditions than any one of its constituents or any two of its constituents combined, the method which comprises heating a major proportion of a lubricating oil, a minor proportion of a friction reducing oil soluble organic compound having oxygen in saponifiable chemical combination therewith, and a minor proportion of another and substantially neutral body of oil film strengthening, oil soluble hydrocarbon having halogen in chemical combination therewith, and homogenizing the mixture with heat until tests 15 on a lubricant tester of samples thereof taken at successive intervals during the heating show maximum and substantially uniform film strength and minimum and uniform friction characteristics.
11. A lubricant compound of high film strength and lower coefficient of friction over a significant range of working conditions than any one of its constituents or any two of its constituents combined, comprising a major proportion of lubricating oil having dissolved therein a minor proportion of a substantially neutral body of oil film strengthening, oil soluble hydrocarbon having a halogen in chemical combination therewith, and a minor proportion of another body of friction reducing, oil soluble organic compound having oxygen in saponifiable chemical combination therewith, said oil, said hydrocarbon and said friction reducing compound being homogenized under anhydrous conditions until samples thereof taken at successive intervals during the homogenizing operation and tested on a lubricant tester show maximum and substantially uniform film strength and minimum and uniform friction.
12. A lubricant compound of high film strength and lower coefficient of friction over a significant range of working conditions than any one of its constituents or any two of its constituents combined, comprising a major proportion of lubricating oil having dissolved therein a minor proportion of a substantially neutral body of oil film strengthening, oil soluble hydrocarbon having a halogen in chemical combination therewith, and a minor proportion of another body of friction reducing, oil soluble organic compound having oxygen in saponifiable chemical combination therewith, said oil, said hydrocarbon and said friction reducing compound being homogenized while heated under anhydrous conditions until samples thereof taken at successive intervals during the heating and tested on a lubricant tester show maximum and substantially unchanging film strength and minimum and unchanging friction.
13. In the manufacture of extreme pressure lubricants in which a halogenated, hydrocarbon, film-strength increasing agent and an oxygen bearing, friction reducing agent are added to a lubricant to increase permanently the lubricating effectiveness thereof, and the halogen and oxy-

gen of said agents are in separate molecules, the method of insuring uniform and maximum effectiveness of the lubricant mixture which comprises heating the basic lubricant and at least 5 one of the added agents under selected conditions of temperature and pressure until tests on a lubricant tester of samples of the complete mixture of the lubricant and added agents prepared from portions taken at successive intervals from 10 the heated mixture during the heating show maximum and substantially uniform film strength and minimum and uniform friction characteristics.

14. In the manufacture of extreme pressure 15 lubricants in which a halogenated, hydrocarbon, film-strength increasing agent and an oxygen bearing, friction reducing agent are added to a lubricant to increase permanently the lubricating effectiveness thereof, and the halogen and 20 oxygen of said agents are in separate molecules, the method of insuring uniform and maximum effectiveness of the lubricant mixture which comprises heating at least one of the ingredients of the mixture until tests on a lubricant tester 25 of samples of the homogenized mixture of all ingredients including the heated ingredient show substantially no change in the film strength and friction characteristics upon further heating of said heated ingredient.

15. In the manufacture of extreme pressure 30 lubricants in which a halogenated, hydrocarbon, film-strength increasing agent and an oxygen bearing, friction reducing agent are added to a lubricant to increase permanently the lubricating effectiveness thereof, and the halogen and 35 oxygen of said agents are in separate molecules, the method insuring uniform and maximum effectiveness of the lubricant mixture which comprises heating and agitating at least two of the 40 ingredients of the mixture until tests on a lubricant tester of samples of the homogenized mixture of all ingredients including the heated and agitated ingredients show substantially no further improvement in the lubricating characteristics of the samples upon further heating 45 of said heated ingredients.

16. A lubricant compound of permanent high film strength and lower coefficient of friction over a significant range of working conditions 50 than any one of its constituents or any two of its constituents combined, comprising a major proportion of lubricating oil having dissolved therein a minor proportion of a halogenated, hydrocarbon film strength increasing agent and an oxygen bearing, friction reducing agent, with the halogen and oxygen in separate molecules, said solution being homogenized while heated until 55 samples thereof taken at successive intervals during the heating and tested on a lubricant tester show substantially no change in lubricating properties.

17. A lubricant compound of permanent high film strength and lower coefficient of friction

over a significant range of working conditions than any one of its constituents or any two of its constituents combined, comprising a major proportion of lubricating oil having dissolved therein a minor proportion of a halogenated, hydrocarbon film strength increasing agent and an oxygen bearing friction reducing agent, with the halogen and oxygen in separate molecules, said solution being agitated and heated until samples thereof taken at successive intervals during the heating and tested on a lubricant tester show substantially no change in lubricating properties. 5

18. A lubricant compound of permanent high film strength and lower coefficient of friction over 15 a significant range of working conditions than any one of its constituents or any two of its constituents combined, comprising a major proportion of lubricating oil having dissolved therein a minor proportion of a halogenated, hydrocarbon 20 film strength increasing agent and an oxygen bearing friction reducing agent, with the halogen and oxygen in separate molecules, at least two of the constituents of said compound being heated, at a temperature at which they remain 25 chemically stable, for such interval that a homogenized mixture of the constituents of the compound including the heated constituents, when tested on a lubricant tester shows unchanging lubricating properties when the mixture is 30 further heated.

19. In the manufacture of extreme pressure lubricants in which a halogenated, hydrocarbon, film-strength increasing agent and an oxygen bearing, friction reducing agent are added to a lubricant to increase permanently the lubricating effectiveness thereof, and the halogen and oxygen of said agents are in separate molecules, the method of insuring uniform and maximum effectiveness of the lubricant mixture which comprises heating the basic lubricant and at least one of the added agents for a minimum period of time depending upon the temperature and varying from a period of approximately 15 minutes at approximately 200° C. to approximately 45 sixteen hours at approximately 110° C. 40

20. In the manufacture of extreme pressure lubricants in which a halogenated, hydrocarbon, film-strength increasing agent and an oxygen bearing, friction reducing agent are added to 50 a lubricant to increase permanently the lubricating effectiveness thereof, and the halogen and oxygen of said agents are in separate molecules, the method of insuring uniform and maximum effectiveness of the lubricant mixture which comprises heating the basic lubricant and at least one of the added agents with agitation for a minimum period of time depending upon the temperature and varying from a period of approximately 15 minutes at approximately 200° C. to approximately 60 sixteen hours at approximately 110° C. 55

WILLIAM ALVAH SMITH.